

## UNITED STATES PATENT OFFICE

WESTON MOREILL, OF PITTSFIELD, MASSACHUSETTS, ASSIGNOR TO GENERAL ELECTRIC COMPANY, A CORPORATION OF NEW YORK

## ALUMINUM ALLOY

No Drawing.

Application filed February 4, 1931. Serial No. 513,455.

The present invention relates to aluminum alloys but more particularly to aluminum alloy castings containing silicon and manganese with or without other metals.

5 It is an object of the present invention to provide a relatively cheap aluminum base alloy which may be cast, have a fair tensile strength, an elongation of approximately 1% in two inches, a low electrical conductivity, and a melting point below 800° C. 10 An alloy of this character is suitable for use as the conducting bars and end rings in induction motor rotors.

15 The alloy forming the subject matter of the present invention preferably consists of the following ingredients:

|              | Per cent |
|--------------|----------|
| Aluminum     | 82.4     |
| Silicon      | 8        |
| 20 Manganese | 8        |
| Copper       | 1        |
| Magnesium    | 0.5      |
| Sodium       | 0.1      |

25 An alloy of this composition has a volume conductivity of about 18% as compared with copper, a tensile strength in the chilled cast state of about 12,500 pounds per square inch, an elongation of about 1% in two inches and a melting point of about 780° 30 C.

The alloy may be manufactured by melting the ingredients in a suitable crucible, for example a crucible made of magnesite or graphite or cast iron the interior of 35 which is limed or whitewashed. The aluminum is first melted and when its temperature is slightly above the melting point, silicon, manganese, copper and magnesium are added so as to give substantially the proportions indicated above in the final product. The molten mass is stirred occasionally until all the ingredients are melted. About 0.1% of sodium is then added to the 40 molten metal. This addition may be made by wrapping the sodium in aluminum foil and plunging it by means of an inverted funnel to the bottom of the molten mass. The temperature is held constant at about 860° 45 C. for approximately five minutes to allow

thorough dissemination of all the constituents and the molten metal then poured into small pigs.

When employed for casting motor rotors the pigs may be remelted in a cast iron pot 55 which has been thoroughly limed but preferably in a graphite crucible. The molten metal is allowed to stand for about five minutes before casting so as to allow all dross to arise to the surface and be removed and 60 to allow the escape of all gases which may be present due to the sodium addition. The desired quantity of liquid molten metal is then removed in a ladle and poured into a centrifugal casting machine or is poured directly from the graphite crucible. 65

If the alloy is to be employed for chill casting, the sodium serves no useful purpose. However, in casting motor rotors, I have found it desirable to preheat the rotor 70 to about 600° C. before casting to ensure that the alloy will completely fill the small conductor bars of the rotor. Under such conditions, if the sodium is absent, the alloy will have a relatively coarse structure. 75 The presence of sodium "modifies" this structure so that slow cooling gives the same final dispersed condition that chilled cooling will give on an alloy containing no sodium. 80

Aluminum alloys are usually "modified" with sodium just before casting. However, to simplify the manufacturing process, I prefer to add sodium to the alloy when it is first made. The remelting eliminates 85 much of the sodium as dross but the original 0.1% provides sufficient excess so that enough sodium remains in the final casting to accomplish "modification".

The present alloy may be employed for 90 any general casting purpose which may require a light weight alloy of low electrical conductivity and not too great strength. The alloy may if desired be cast at slow speed in a centrifugal machine or with no rotation 95 whatever.

While manganese aluminum alloys have been employed heretofore in the manufacture of motor rotors, such alloys are not entirely satisfactory since a manganese alumi- 100

num compound appears to separate out in large cubes throughout such metal thereby weakening it to a great extent. Silicon has approximately the same specific gravity as aluminum and, when present in substantially equal quantities with manganese in an aluminum alloy, the silicon keeps the manganese in a finely dispersed condition providing a fine grain uniform composition in which there is no segregation of the components in the cast product.

While I prefer to employ an alloy containing about 8% manganese and 8% silicon with the remainder aluminum, my invention is not limited to these specific quantities. The manganese and silicon are employed in substantially equal amounts which, for each of these ingredients, may vary from about 4% to about 13%. The lower quantity of silicon and manganese (4% each) provides an alloy having a tensile strength of about 19,000 pounds per square inch and a conductivity of about 24.4%, while the alloy with the higher silicon and manganese content (13% each) provides an alloy having a tensile strength of 10,500 pounds per square inch and a conductivity of about 12.5%.

Although I usually employ in the alloy about 1% copper, 0.5% magnesium and 0.1% sodium, these ingredients are not absolutely essential. They affect the physical properties of the alloy somewhat but may generally be omitted without adversely affecting its properties. If desired, the alloy may contain up to 4% copper.

The alloy may be strengthened and its elongation increased by the addition of a small amount of silver, for example 1%. The addition of silver has but little effect on the electrical conductivity of the alloy, but of course increases its cost.

What I claim as new and desire to secure by Letters Patent of the United States, is:

1. An alloy containing about 8% manganese, about 8% silicon, the remainder of the alloy consisting substantially of aluminum.

2. An alloy containing from 4 to 13% manganese, 4 to 13% silicon, the remainder of the alloy consisting substantially of aluminum.

3. An alloy containing about 82.4% aluminum, about 8% silicon, about 8% manganese, approximately 1% copper, 0.5% magnesium and 0.1% sodium.

In witness whereof, I have hereunto set my hand this 28th day of January, 1931.

WESTON MORRILL.